# EUROPEAN PATENT APPLICATION

(11) **EP 0 638 335 A1**
(43) Date of publication of application: **15.02.1995**
(21) Application number: 94305374.4
(22) Date of filing: 20.07.1994
(51) Int. Cl.: A62D 1/00

(54) **Deflagration suppression agent and method for its use**

(30) Priority: 02.08.1993 US 100395
(71) Applicant: FENWAL SAFETY SYSTEMS, INC., Marlboro, Massachusetts 01752 (US)
(72) Inventor: Senecal, Joseph A., Massachusetts 02181 (US)
(74) Representative: Thomson, Paul Anthony

(57) **Abstract**

A deflagration suppression agent consisting of a dry powdery material composed of nonflammable particles each providing a surface area capable of rapidly absorbing heat and thereby cooling a deflagration reaction zone, and wherein at least 90% of the particles have a mean diameter of less than 20 microns.

## Description

### BACKGROUND OF THE INVENTION

This invention relates generally to a suppression agent, and more particularly, to a powdery suppression agent for effectively extinguishing a flame front of a developing deflagration.

Nonflammable powdery materials are used commonly as fire extinguishing agents. Generally, such agents are used to fill portable fire extinguishers that can be manually transported from a storage position to a region in which a fire has ignited. Most commercially available fire extinguishing powders consist primarily of relatively large particles having mean diameters of, for example, greater than 100 microns. Although the fire extinguishing efficiency of very small particles (VSPs) is known, high concentrations of VSP materials have not been employed as dry chemical fire extinguishing products because of inherent properties which are detrimental in typical fire extinguishing applications. Among these detrimental properties are high cost; low bulk density requiring larger, heavier and more costly containers and reduced "throw" which limits the effective range of a discharged powder stream. In addition, VSPs have the inherent characteristic of exhibiting a high degree of airborne persistence which is undesirable for fire extinguishing applications in which a desired objective is to coat flammable surfaces. Such coating of surfaces both extinguishes fire thereon and prevents the spread of flame. Because typical fires exist on surfaces, airborne suppression materials have little extinguishing effectiveness.

The object of this invention is to provide an improved dry powdery agent that will rapidly and effectively suppress developing deflagrations.

### SUMMARY OF THE INVENTION

The invention is a deflagration suppression agent consisting of a dry powdery material composed of nonflammable particles each providing a surface area capable of rapidly absorbing heat and thereby cooling a deflagration reaction zone, and wherein at least 90% of the particles have a mean diameter of less than 20 microns. Effective suppression of a deflagration is provided by the very small particles which enhance the extinguishing function per unit mass of material.

According to specific features of the invention, the material is either silica, aluminum oxide, titanium oxide or combinations thereof. These materials exhibit ideal characteristics for the suppression function.

According to another feature of the invention, 90% of the particles have a mean diameter less than 5 microns. Suppression effectiveness is enhanced further by a reduction in particle size.

The invention also encompasses a method for the suppression of a deflagration and includes the steps of: determining a deflagration reaction zone; filling a container having a discharge opening with a dry powdery material composed of nonflammable particles, at least 90% of the particles having a mean diameter less than 20 microns; pressuring the container with a gas; disposing the container in a position that directs the discharge opening toward the reaction zone; detecting a flame front of a developing deflagration in the reaction zone; and releasing the dry powdery material and gas through the discharge opening and into the reaction zone. Release of the very small particles into the reaction zone quickly extinguishes the detected flame front to terminate a developing deflagration.

### DESCRIPTION OF THE PREFERRED EMBODIMENTS

An extinguishant for suppressing deflagrations consists of a dry powdery material primarily composed of nonflammable very small partices (VSPs) which improve deflagration suppression efficiency by providing high specific surface area and consequent ability to absorb heat and thereby cool a deflagration reaction zone to a temperature which will not support the chemical reactions required to maintain a flame front. In addition, the small particles exhibit a tendency to remain airborne in the deflagration reaction zone thereby inhibiting any tendency for flame reignition to occur. Preferably, at least 90% of the particles constituting the suppression agent have a mean diameter of less than 20 microns and even further suppression efficiency is obtained by a suppression agent composed of particles of which at least 90% have a mean diameter of less than 5 microns. Suitable nonflammable dry powdery materials include silica, aluminum oxide and titanium oxide. The selected powdery agents, either alone or in a predetermined combination, are subjected to a classification procedure to obtain an agent mixture having the desired critical particle size distribution.

In preferred methods of use, the suppression agents are used in deflagration suppression systems employing high rate discharge (HRD) extinguishers. Such extinguishers include highly directional discharge openings closed either by quick acting valves or explosively activated frangible closures. The extinguishers are filled with the dry powdery agent and then pressurized with a suitable gas such as nitrogen or gases such as carbon dioxide or tryfloromethane which can themselves contribute to enhanced suppression efficiency.

After being charged with a dry powdery suppression agent and pressurized gas, the extinguisher is mounted in a position that directs it's discharge opening toward a previously determined deflagration reaction zone. Typically such zones are located in enclosures that process materials capable of providing mixtures that can support a deflagration. The deflagration reaction zone usually will be within a few feet of the extinguisher discharge opening so as to render the relatively low density and "throw" capability of the VSP agent inconsequential.

Upon detection of a flame front of a developing deflagration by a suitable detector, the extinguisher is activated to release the dry powdery agent and gas through the discharge opening and into the reaction zone wherein the VSPs rapidly absorb heat to cool the reaction zone to a temperature below that required to support the propagation of a flame front and resulting in suppression. Suitable deflagration suppression systems for use with the VSP agents of the invention are disclosed, for example, in U.S. Patent No. 4,487,266 and U.S. Patent Application Serial No. 06/344,531.

Obviously, many modifications and variations of the present invention are possible in light of the above teachings. It is to be understood, therefore, that the invention can be practiced otherwise than as specifically described.

## Claims

1. A deflagration suppression agent comprising:
a dry powdery material composed of nonflammable particles each providing a surface area capable of rapidly absorbing heat and thereby cooling a deflagration reaction zone, and wherein at least 90% of said particles have a mean diameter of less than 20 microns.

2. A deflagration suppression agent according to claim 1 wherein said material comprises particles of silica.

3. A deflagration suppression agent according to claim 1 wherein said material comprises particles of aluminum oxide.

4. A deflagration suppression agent according to claim 1 wherein said material comprises particles of titanium oxide.

5. A deflagration suppression agent according to claim 1 wherein 90% of said particles have a mean diameter less than 5 microns.

6. A deflagration suppression agent according to claim 5 wherein said material comprises particles of silica.

7. A deflagration suppression agent according to claim 5 wherein said materail comprises particles of aluminum oxide.

8. A deflagration suppression agent according to claim 5 wherein said material comprises particles of aluminum oxide.

9. A method for the suppression of a deflagration which comprises the steps of:
determining a deflagration reaction zone;
filling a container having a discharge opening means with a dry powdery material composed of nonflammable particles, at least 90% of said particles having a mean diameter less than 20 microns;
pressuring said container with a gas;
disposing said container in a position that directs said discharge opening toward said reaction zone;
detecting a flame front of a developing deflagration in said reaction zone; and
releasing said dry powdery material and gas through said discharge opening means and into said reaction zone.

10. A method according to claim 9 wherein said material comprises particles of silica.

11. A method according to claim 10 wherein said material comprises particles of aluminum oxide.

12. A method according to claim 11 wherein said material comprises particles of titanium oxide.

13. A method according to claim 9 wherein 90% of said particles have a mean diameter less than 5 microns.

14. A method according to claim 13 wherein said material comprises particles of silica.

15. A method according to claim 14 wherein said material comprises particles of aluminum oxide.

16. A method according to claim 15 wherein said material comprises particles of titanium oxide.
